

## UNITED STATES PATENT OFFICE

2,454,823

VISCOSITY REDUCTION OF PETROLEUM  
MAHOGANY SULFONATE HYDROCAR-  
BON SOLUTIONSAbraham Moscowitz, New York, N. Y., assignor to  
L. Sonneborn Sons, Inc., a corporation of Dela-  
wareNo Drawing. Application November 21, 1946,  
Serial No. 711,476

8 Claims. (Cl. 260—504)

1

This invention relates to new and useful improvements in the viscosity reduction of petroleum mahogany sulfonate hydrocarbon solutions. Petroleum mahogany sulfonate solutions in organic solvents of the water immiscible type are used for a variety of purposes such as wetting agents, emulsifying agents and the like. Ordinary petroleum mahogany sulfonates impart to their solutions a relatively high viscosity. In some cases this high viscosity is not critical regarding the purpose for which the sulfonate solutions are to be used. There are, however, many cases in which a relatively high viscosity is undesirable or detrimental to their intended use or application. This is, for example, true in textile processing such as of wool, worsted, rayon, viscose or the like in which the various processing steps involved in the conversion of the raw materials into fibres, the formation of the fibres into threads and the weaving of the threads into fabric, require the presence of a lubricating agent having a Saybolt viscosity of below 600 and preferably below 300 seconds Saybolt at 100° F. The latter is particularly true of textile lubricants used in the processing of synthetic fibres. In the case of textile processing it is for instance desirable to have a hydrocarbon textile lubricant composition with a sulfonate content of in excess of 28% mahogany sulfonate so as to render the composition not only readily and spontaneously emulsifiable but also to make the same readily wettable or rewettable on the fibre to thereby impart to the textile material substantial self-scourability. Hydrocarbon solutions of the textile lubricant type and containing in excess of 28% of petroleum mahogany sulfonates possess, however, a viscosity far in excess of 600 seconds Saybolt at 100° F. and usually a viscosity in excess of 1000 seconds Saybolt at 100° F. For this reason it has been in the past necessary in such cases to limit the sulfonate content to a maximum of approximately 15% in order not to exceed the usable viscosity for textile material treating purposes. Another example is the use of petroleum mahogany sulfonates in the compounding of cutting oil bases in which the relatively high viscosity and tackiness imparted to the composition by the sulfonates is an undesirable aspect interfering in many respects with the proper ease of application and use.

The relatively high viscosity of petroleum mahogany sulfonates in organic solvents is normally not subject to reduction by the addition of relatively low viscous diluents or thinning agents. This requires agents of such relatively low vis-

cosity that they interfere with the lubricating properties of the composition. Furthermore, these solvents are then of the type which easily evaporate. This is particularly critical in the case of textile treating materials since the use of such thinning solvents will leave behind on the fibre upon evaporation a viscous sticky impregnant without adequate lubricating capacity on the fibre and will also interfere with the scourability of the impregnated material. On the other hand thinning with a solvent of the lubricant type diluent will not obtain the desired result as it is necessary to add so much of the diluent as to bring the sulfonate content to below that necessary for adequate emulsification or other purpose for which the composition is designed.

Certain treatments of petroleum mahogany sulfonate hydrocarbon solutions with hypochlorites or chlorites are accompanied by a viscosity reduction. Thus for instance a viscosity reduction is obtained by subjecting a petroleum sulfonate product dissolved in a hydrocarbon, including a hydrocarbon of the mineral oil type (for example "retained" oil conventionally derived from the acid refining of a petroleum oil distillate) to a treatment with sodium hypochlorite or sodium chlorite until a Lovibond value of less than 8R and preferably about 2-3R (10% while oil solution  $\frac{1}{2}$ " cell) is obtained. This is, for instance, set forth respectively in U. S. Patent 2,201,119 issued to M. Blumer et al., and U. S. Patent 2,307,743 issued to L. Liberthson et al. The hypochlorite treatment requires relatively large amounts of hypochlorite for which reason undesirably large amounts of inorganic salts may be produced as a result of the reaction, necessitating salt removal purification. Furthermore, in many cases the hypochlorite treatment does not produce as efficient or as low a viscosity reduction as may be desired. This would apply, for instance, where a petroleum mahogany sulfonate textile lubricant composition is to be used for synthetic fibre processing, in which case a viscosity below 300 seconds Saybolt at 100° F. for a sulfonate content of in excess of 28% is desirable. On the other hand, the chlorite treatment, though somewhat more effective in viscosity reduction of suitable petroleum mahogany sulfonate hydrocarbon solutions, has to be carried out at an acid pH and necessitates neutralization of the resultant chlorite-treated product. Such neutralization, however, is in many cases accompanied to some extent by a viscosity reversion, i. e., an increase of the viscosity from that of the acidified treated solu-

tion. This viscosity increase negatives, at least to some degree, the viscosity decrease effected by the chlorite reaction. Though this reversion can be kept in most cases sufficiently low so that the resultant neutralized product still possesses an appreciably lower viscosity than the untreated mahogany sulfonate composition, the reverted viscosity may yet be undesirably high for many purposes.

I have discovered that it is possible to obtain a viscosity reduction of a petroleum mahogany sulfonate organic solvent solution which is more efficient than either the hypochlorite or chlorite treatment, and will permit the reaction to be carried out at an acid or alkaline pH. If carried out at an alkaline pH the disadvantage of viscosity reversion upon neutralization from an acid pH is completely eliminated. If operating at an acid pH such viscosity reversion in this case is relatively negligible. At the same time when proceeding in accordance with my discovery it is possible to operate in such a manner that such inorganic residue as may be produced by reason of the treatment is relatively small and may in many cases be disregarded without substantially impairing the functions or properties of the sulfonate in solution for the particular composition for which it is desired. In this manner inorganic salt removal or purification is unnecessary.

In accordance with the invention a suitable petroleum mahogany sulfonate solution in an organic substantially water immiscible solvent for said sulfonate is reacted with an alkali metal chlorite and an alkali metal hypochlorite in amount and for a period of time sufficient to appreciably reduce the normally relatively high viscosity of said solution due to the sulfonate dissolved therein and preferably reduce said viscosity by at least one-third.

The solvents that may be used for this purpose should be substantially neutral to chlorite and/or hypochlorite action, should not appreciably dissolve inorganic salts and should be substantially liquid at normal temperatures. Suitable solvents that may be used in the practice of the invention are, for instance, petroleum oil distillates or any fraction thereof, benzol and its homologs, naphtha, carbon tetrachloride, tetrachlorethane, chloroform, etc., and in general any aromatic or aliphatic or aryl or aralkyl hydrocarbon or hydrocarbon mixture including their halogenated derivatives of the aforescribed character and nature. In many cases, particularly where the solvent is to be removed after the viscosity reducing treatment, it is desirable to have the boiling range of such solvent sufficiently low to permit removal in the customary manner such as by distillation in vacuo or otherwise without causing thereby any decomposition of the mahogany sulfonates. In such cases it is of advantage that the boiling point be so low and preferably between 75 and 250° F. as to enable the removal of the solvent at ordinary temperatures without the necessity of resorting to vacuum distillation.

The petroleum mahogany sulfonate which is subjected to the viscosity reduction is normally one derived from the acid refining, with fuming sulfuric acid, of a petroleum oil distillate stock under sulfonating conditions of acid amount and temperature in accordance with conventional refining practice. In such conventional fuming sulfuric acid refining an oil layer and acid sludge layer are formed, the former containing dissolved therein petroleum mahogany sulfonic acids col-

lectively referred to as mahogany petroleum sulfonic acids. These are recovered from the oil layer in accordance with conventional methods in the form of solutions of these sulfonic acids or their salts (the latter being collectively termed "petroleum mahogany sulfonates") in a portion of the oil relatively tenaciously occluded by these sulfonic bodies. This occluded oil is generally referred to in the art as "retained" oil. The petroleum sulfonic acids or sulfonate oil compositions normally contain about 30 to 35% of retained oil and 65 to 70% of the petroleum mahogany sulfonic material. Depending upon the type and origin of petroleum oil distillates from which these sulfonate-oil solutions or stocks are derived they contain sulfonates of varying averaged molecular weights. For convenience therefore the sulfonate stocks are identified by their average molecular weights. Thus, a 420 or 450 sulfonate stock is a stock in which the sulfonates have an average molecular weight of 420 or 450 respectively.

It is possible to carry out the chlorite-hypochlorite reaction at either an alkaline or acid pH. Excess alkalinity or acidity should be avoided, however, as they are detrimental to the efficiency of the viscosity reduction and may furthermore give rise to partial decomposition of the sulfonates and an undesirable color deterioration rather than color improvement in the resultant products. For reasons of viscosity reversion upon neutralization, though relatively small, it is preferred to carry on the chlorite-hypochlorite treatment at a neutral to alkaline pH and within the preferred embodiment of the invention a pH range from 7.5 to 8.5 is recommended.

In the practical application of the invention, a suitable petroleum mahogany sulfonate solution is intimately contacted with an alkali metal chlorite and an alkali metal hypochlorite. In the preferred mode of such treatment 1.5 to 7% and preferably 2.5 to 6% of the chlorite and hypochlorite (calculated on the aggregate dry weight by weight of sulfonate in solution) are used in a proportion of 0.5 to 4 parts by weight and preferably of 2 to 3 parts by weight of hypochlorite for every one part by weight of chlorite. The reaction is continued until the desired viscosity reduction is obtained. If necessary, the solution may be acidified with  $H_2SO_4$  to the desired pH range. The preferred procedure is to dissolve the chlorite in the aqueous hypochlorite solution.

The temperature of reaction is ordinarily not critical. The reaction, however, may be facilitated by increasing the temperature to for example a preferred temperature of from 120 to 200° F. This is particularly desirable with more heavily viscous solutions as the higher temperature will increase the fluidity of the solution, thus permitting more intimate contact between the reactants.

The extent to which low viscosity values may be obtained depends, at least to some extent, upon the type or origin of the petroleum mahogany sulfonate selected for the treatment. Ordinarily higher average molecular weight sulfonates possess a higher viscosity and the resulting viscosity after treatment is usually commensurately higher than the viscosity after treatment of a comparative sulfonate hydrocarbon solution which before treatment possessed a relatively lower viscosity and in which the sulfonate had a lesser average molecular weight.

The ratio of petroleum mahogany sulfonate to solvent is, as a rule, not critical except that it is desirable to so adjust the ratio that the viscosity

of the solution is sufficiently low at the desired or selected temperature of treatment to permit the intimate contact between the reactants. In most cases, however, a ratio of mahogany sulfonate to solvent of substantially 2 to 1 (by weight) will give satisfactory results. Sulfonate concentrations above 70 to 75% sulfonate content are normally not desirable for direct reaction without suitable extension. As a mode of agitation, any conventional method such as stirring, air-blowing, shaking, etc. may be used.

As above pointed out, the viscosity reducing reaction in accordance with the invention may be carried out with an organic solvent solution containing relatively high concentrations of petroleum mahogany sulfonate. In this case the resultant product is a concentrate which in many cases must be thereafter adjusted by the addition of organic solvent material of suitable viscosity, such as a suitable lubricant hydrocarbon, to the requisite petroleum mahogany sulfonate content desired for the specific purpose for which the composition is to be used. Thus, for instance, if it is desired to ultimately produce a textile treating oil having in excess of 28% petroleum mahogany sulfonate and a viscosity of less than 600 seconds Saybolt at 100° F., a concentrate having in excess of 40% and usually between 60 and 65% sulfonate, is first obtained after the viscosity reducing reaction in accordance with the invention, which product may be then extended by the addition of a suitable lubricant hydrocarbon such as a mineral pale oil having a viscosity of 75 seconds Saybolt at 100° F. to a sulfonate content between 28 and 40% and a viscosity below 600 seconds Saybolt at 100° F.

Alternatively, the viscosity reducing reaction may be carried out with an organic solvent solution of a petroleum mahogany sulfonate already possessing the requisite final sulfonate content desired and intended for the purpose for which the viscosity reduced product is to be used. In that case it is also of advantage to select for the solution such solvent as is desired for the final product, i. e., if a textile lubricating oil is intended to be ultimately obtained a textile lubricant, having, for instance, a viscosity between 40 and 150 seconds Saybolt at 100° F. is selected as the solvent for the sulfonate. The product resulting from the viscosity reducing treatment is then per se usable after such further refining or purification as may be required for a textile treating oil.

Though in the operation of the novel viscosity reducing process any of the aforementioned solvents may be used with advantage, I prefer to use as the solvent that hydrocarbon fraction, the acid refining of which furnished the crude mahogany sulfonate stock and which is carried as "retained" oil. The crude mahogany sulfonate-retained oil stock constitutes as such a convenient mahogany sulfonate solution that may be subjected directly to treatment in accordance with the invention.

Instead of adding in the operation of the invention hypochlorite per se as a component of the hypochlorite-chlorite combination, it is possible, if desired, to produce the hypochlorite or other hypochlorous equivalent in situ in the solution through the stoichiometric interaction of chlorine and an aqueous and/or alkaline medium.

Whenever carrying out the viscosity reducing procedure in accordance with the invention in a manner yielding directly a usable product of a sulfonate content reduced viscosity and type of solvent per se usable for a predetermined purpose, this may be also accomplished by a modifi-

cation of the conventional acid refining. In this case the solvent is necessarily the oil, the acid refining of which will furnish the mahogany sulfonate stock. When proceeding in this manner a petroleum oil distillate is given at a temperature of about 150° F., a 50% batch treatment with fuming sulfuric acid, i. e., a treatment (sometimes in several batches) with 50% of acid by weight of the oil treated. The cooled acidified oil is thereafter diluted with an equal volume of benzol or benzol homolog, the mixture is permitted to settle overnight and the acid sludge layer is withdrawn. After neutralizing the oil layer and removing the benzol by distillation, the oil layer is subjected to the viscosity reducing reaction in accordance with the invention. The resulting product contains approximately 30% of petroleum mahogany sulfonates, about 70% of lubricant mineral oil (of the textile lubricant usable type) and possesses a viscosity below 600 seconds Saybolt at 100° F. Once a petroleum mahogany sulfonate has been subjected in suitable solvent medium to a viscosity reducing reaction in accordance with the invention, it is possible to remove the solvent if desired and recover the petroleum mahogany sulfonates as such substantially free from solvent. These sulfonates when redissolved in the solvent still exhibit in solution the same reduced viscosity which they possessed prior to the removal of the solvent.

The following examples are furnished by way of illustration and not of limitation.

*Example I*

35 100 lbs. of petroleum sulfonate-retained oil stock (containing 61-2% sodium sulfonates) were heated to 120° F.; a solution of 1 lb. sodium chlorite in 5 lbs. aqueous hypochlorite solution having a 10% available chlorine content was added. 40 The mixture was heated to 200° F. and maintained at this temperature, while stirring, for one-half hour, then blown with air to drive out retained moisture and diluted with 75 viscosity mineral oil to a 30% sulfonate content. Before treatment, the petroleum sulfonate-retained oil stock had a viscosity of 163 furol at 210° F. and upon dilution to a 30% sulfonate content 1463 Saybolt at 100. After treatment and before dilution the corresponding viscosity was 113 furol at 210° F. and after dilution 375 Saybolt at 100° F.

*Example II*

55 100 lbs. of a petroleum mahogany sulfonate stock containing 61-2% sulfonate and 38% retained oil was used. The stock was obtained from a Mid-Continent distillate subjected to white oil refining with fuming sulfuric acid under sulfonating conditions. The mahogany sulfonates in the stock possessed an average molecular weight of 450, a furol viscosity of 144 seconds at 210° F. and a Lovibond color value of about 8R (10% white oil solution  $\frac{1}{2}$ " cell). 1 lb. of sodium chlorite was dissolved in 2.5 lbs. of an aqueous sodium hypochlorite solution having an available chlorine content of approximately 10%. This chlorite-hypochlorite solution was then added to the sulfonate stock, whereupon the mix was agitated, maintaining the temperature at about 180 to 200° F. The pH was adjusted to about 8 and the treatment was continued until a sample showed a reduced Lovibond color (10% white oil solution  $\frac{1}{2}$ " cell) of about 2-3R, which was achieved after about one-half hour. After treatment the reduced viscosity was 73 furol at 210° F. and after dilution with a mineral pale oil (75

—seconds Saybolt at 100° F.) to a 30% sulfonate content a viscosity of 400 seconds Saybolt at 100° F.

*Example III*

100 lbs. of a Mid-Continent distillate containing about 30 to 35% sulfonatables was treated at about 150° F. with about 50 lbs. of fuming sulfuric acid. After completion of the addition of the

and 40% sulfonate content respectively as against the viscosities of the same stock treated in accordance with the invention and of 30%, 35% and 40% sulfonate content dilutions for each treated stock. The treatment of each stock was carried out as specified in Examples I or II. The extending oil in each case was a neutral solvent refined mineral pale oil having a Saybolt viscosity of 75 or 50 seconds at 100° F. as specified.

| Type of Sulfonate Stock |            | Per Cent Sodium Sulfonate | Furol Vis. at 210° F. | Saybolt Viscosities at 100° F. When Extended With 75 vis. neutral to Sodium Sulfon. Cont. |       |       | Viscosity Reduction Obtained by— |                       |     |     |     |     |     |
|-------------------------|------------|---------------------------|-----------------------|-------------------------------------------------------------------------------------------|-------|-------|----------------------------------|-----------------------|-----|-----|-----|-----|-----|
|                         |            |                           |                       |                                                                                           |       |       | Furol Vis. at 210° F.            | Chlorite—Hypochlorite |     |     |     |     |     |
| Av. Mol. Wt.            | Source     | 30%                       | 35%                   | 40%                                                                                       | 30%   | 35%   | 40%                              | 30%                   | 35% | 40% | 30% | 35% | 40% |
| 500                     | Gulf Coast | 62                        | 205                   | 1,500                                                                                     | 1,750 | 2,100 | 110                              | 475                   | 550 | 590 | —   | —   | —   |
| 450                     | Mid. Cont. | 62                        | 144                   | 1,100                                                                                     | 1,280 | 1,475 | 73                               | 400                   | 495 | 575 | —   | —   | —   |
| 420                     | Penna.     | 62                        | 81                    | 910                                                                                       | 1,050 | 1,200 | 39                               | 380                   | 475 | 560 | 185 | 240 | 285 |

acid, the oil was permitted to cool and the cooled, acidified oil was thereafter diluted with an equal volume of benzol. The mixture was then permitted to settle overnight, whereupon the acid sludge layer was withdrawn. The oil layer was then neutralized with an aqueous caustic solution of about 27° Bé. After settling the aqueous spent caustic layer was removed, whereupon the oil-benzol layer was subjected to distillation for the removal of the benzol. There was then added to the resulting mahogany petroleum hydrocarbon solution a chlorite-hypochlorite solution prepared by dissolving 0.5 lb. of sodium chlorite in 1.25 lbs. of aqueous sodium hypochlorite solution (having an available chlorine content of approximately 10%). The mix was agitated, the temperature maintained at about 180 to 200° F. and the pH adjusted to about 8. The temperature and agitation were continued until a sample showed a reduced Lovibond color of about 2-3R, which result was achieved after about one-half hour. The resulting stock contained approximately 70% of petroleum hydrocarbon oil, about 30% of petroleum mahogany sulfonates, and possessed a viscosity substantially of about 410.

*Example IV*

50 lbs. of the same 62% sulfonate stock specified in Example II were extended with 52 lbs. of a 75 seconds Saybolt viscosity (at 100° F.) pale oil to yield a 30% sulfonate content. There was then added to the resultant product having a viscosity of 1100 seconds Saybolt at 100° F., 0.5 lb. sodium chlorite dissolved in 1.25 lbs. of an aqueous sodium hypochlorite solution (10% available chlorine content). The chlorite-hypochlorite combination was added while the mix was agitated and the temperature brought to about 180 to 200° F. The pH of the mix was adjusted to about 8 and agitation and the temperature continued until the sample showed a reduced Lovibond color of about 2-3R, which was obtained after about one-half hour. The resultant product contained about 30% petroleum mahogany sulfonate, about 70% mineral oil and a viscosity of about 390 seconds Saybolt at 100° F.

In the following table comparative viscosity data are furnished of various sulfonate stocks showing in each case the viscosities of the untreated stock and of dilutions thereof to 30, 35

The foregoing description is for purposes of illustration and not of limitation and it is therefore my intention that the invention be limited only by the appended claims or their equivalents 30 wherein I have endeavored to claim broadly all inherent novelty.

I claim:

1. Process for reducing the viscosity of petroleum mahogany sulfonate solutions, which comprises treating a petroleum mahogany sulfonate solution in an organic substantially water-immiscible solvent for said sulfonate with an alkali metal chlorite and an alkali metal hypochlorite in a proportion of 0.5 to 4 parts by weight of hypochlorite for every 1 part by weight of chlorite and in amount and for a period of time sufficient to appreciably reduce the normally relatively high viscosity of said solution due to the sulfonate dissolved therein.

2. Process in accordance with claim 1 in which the treatment is carried out with an amount of chlorite and hypochlorite and for a period of time sufficient to reduce said normally relatively high viscosity of said solution by at least one-third.

3. Process in accordance with claim 1 in which said solution is treated with said sodium chlorite and hypochlorite combination in amount and for a period of time sufficient to yield a reduction to a Lovibond color value below 8R.

4. Process in accordance with claim 1 in which said solution is treated with said sodium chlorite and hypochlorite combination in amount and for a period of time sufficient to yield a reduction to a Lovibond color value of about 2-3R.

5. Process for reducing the viscosity of petroleum mahogany sulfonate solutions, which comprises treating a petroleum mahogany sulfonate solution in an organic substantially water-immiscible solvent for said sulfonate with 1.5 to 7% aggregate dry weight of alkali metal chlorite and alkali metal hypochlorite by weight of sulfonate in solution in a proportion of 0.5 to 4 parts by weight of hypochlorite for every one part by weight of chlorite.

6. Process in accordance with claim 5 in which said chlorite-hypochlorite treatment is carried out at a pH of from 7 to 8.5.

7. Process for reducing the viscosity of petroleum mahogany sulfonate solutions, which com-

prises treating at a pH of from 7 to 8.5, a petroleum mahogany sulfonate solution in an organic substantially water-immiscible solvent for said sulfonate with an aqueous solution of 1.5 to 7% aggregate dry weight of alkali metal chlorite and alkali metal hypochlorite by weight of sulfonate in solution in a proportion of 0.5 to 4 parts by weight of hypochlorite for every one part by weight of chlorite.

8. Process in accordance with claim 7 in which said aqueous solution contains said chlorite and hypochlorite in a ratio of 2 to 3 parts by weight of hypochlorite for every one part by weight of chlorite.

ABRAHAM MOSCOWITZ. 15

10  
REFERENCES CITED  
The following references are of record in the file of this patent:

UNITED STATES PATENTS

| Number    | Name          | Date          |
|-----------|---------------|---------------|
| 2,201,119 | Blumer et al. | May 14, 1940  |
| 2,307,743 | Libirthson    | Jan. 12, 1943 |

OTHER REFERENCES

Article from Technical Assn. Papers—1940—  
"Use of Sodium Chlorite in Bleaching" by Taylor  
et al., pages 251-256.